

# UNITED STATES PATENT OFFICE.

HUGH MACKAY, OF EL PASO, TEXAS.

## LEATHER PRODUCT AND PROCESS FOR MAKING THE SAME.

No. 911,140.

Specification of Letters Patent.

Patented Feb. 2, 1909.

Application filed September 23, 1907. Serial No. 394,161. (Specimens.)

*To all whom it may concern:*

Be it known that I, HUGH MACKAY, a citizen of the United States, and a resident of El Paso, in the county of El Paso and 5 State of Texas, have invented a new and Improved Leather Product and Process for Making the Same, of which the following is a full, clear, and exact description.

My invention relates to the treatment of 10 sole leather, my particular object being to increase the durability and wearing capacity of sole leather, and also to increase the weight of the leather while changing its general character for the better. Briefly 15 stated, I complete the leather, after the tanning process is completed, by causing a composition to become absorbed in the pores. I have found, however, that my process is 20 equally efficacious when applied to leather which has been only partially tanned or which is undergoing the process of tanning, as well as that in which the tanning is complete.

I take leather, for instance ordinary sole 25 leather, and soak it in water until it becomes thoroughly pliant. I then take it out of the water and allow it to become about half dry. I then color the leather in any approved manner and give it a good coating of boiled 30 linseed oil applied upon the grain side only of the leather. This coating I let dry in thoroughly. I next prepare a bath by mixing together Portland cement, borax and cold water in the proportion of eight ounces 35 of cement, two ounces of borax and enough water to reduce the mixture to the consistency of milk. I then place the leather in the bath, allowing one pound of the leather to so much of the bath as contains 40 one half pound of the Portland cement and borax in a dry state.

The preparations stated are somewhat arbitrary, and may be varied within reasonable limits.

45 I allow the leather to stay in the bath for twenty-four hours, after which I remove the leather and examine it, preferably by cutting its edge. If the mixture has not permeated the pores of the leather, I return the same 50 to the bath. The longer the leather remains in the bath, the firmer and heavier it becomes. When the substance of the leather has reached a proper consistency, I remove the leather and allow it to dry. When it 55 becomes nearly dry, I give it a good coat of linseed oil, applied upon both sides of the

leather. When the leather is dry, I roll and finish it, thereby completing it for use.

I find that sole leather treated as above described has its durability increased from 60 one hundred to two hundred per cent. as compared with leather not so treated; and furthermore, that the process renders the leather waterproof.

The details of the process may be varied 65 slightly without deviating from the spirit of my invention. For instance the coloring of the leather and the coating thereof with linseed oil may in some instances be dispensed with. So also the composition of the 70 completed product may be varied slightly in accordance with the preparations employed in the tanning process.

I find further that objects made of heavy 75 leather not requiring any great degree of flexibility, may be treated in accordance with the process substantially as above described, and that the leather or analogous material is improved in like manner as sole leather. It matters not whether the process 80 be employed in connection with the complete leather or with leather partially finished at some previous time, or with leather in the process of tanning. The improvement appears to be equally efficacious in all cases. 85 When shoe soles are treated as above described, there is no injury whatever to either thread, pegs or nails.

Having thus described my invention, I 90 claim as new and desire to secure by Letters Patent:

1. The process herein described of surface hardening sole leather which consists in soaking the same in an aqueous mixture of Portland cement and borax. 95

2. The method herein described of surface hardening sole leather which consists in closing the pores of the same with Portland cement and borax for the purpose of increasing the durability of said leather. 100

3. The process herein described of surface hardening sole leather which consists in soaking the same, for the purpose of opening the pores, preparing a bath containing Portland cement, borax and water, soaking said leather in said bath, and afterwards drying said leather and coating both sides with oil. 105

4. The leather product herein described consisting of leather the pores of which contain Portland cement. 110

5. The process of treating sole leather which consists in soaking the same in water,

partially drying the soaked leather, coating the grain side of the partially dried leather with linseed oil and allowing the oil to dry, preparing a bath containing Portland cement, borax and water, soaking the partially treated leather in said bath, again partially drying said leather and coating both sides of the leather with linseed oil.

In testimony whereof I have signed my name to this specification in the presence of 10 two subscribing witnesses.

HUGH MACKAY.

Witnesses:

H. A. DONNELLY,  
WILBUR SNOW.